

## UNITED STATES PATENT OFFICE.

JAMES H. GRAVELL, OF ELKINS PARK, PENNSYLVANIA.

## MATERIAL AND PROCESS FOR PREPARING METAL FOR PAINTING.

No Drawing.

Application filed January 20, 1923. Serial No. 614,042.

*To all whom it may concern:*

Be it known that I, JAMES H. GRAVELL, a citizen of the United States, residing at Elkins Park, in the county of Montgomery and State of Pennsylvania, have invented a new and useful Improvement in Materials and Processes for Preparing Metal for Painting, of which the following is a specification.

10 This invention relates to improvements in the preparation of metal for painting and more particularly to the preparation for painting of metal articles which, due to their size or shape, are not adapted for immersion in a chemical bath but are susceptible to being brushed, sprayed, scrubbed or similarly treated with a chemical wash.

20 The object of the invention is to remove dirt, scale, rust and material that causes rust in a simple and effective manner so that when that work is completed the metal will be in a condition suitable for receiving a protective coating of paint or the like. By a slight modification of the invention the 25 material and process may be adapted to remove oil in addition to the substances already mentioned from metal surfaces.

Generally stated, the invention consists in applying an acid colloidal wash, herein-30 after more fully described, to the surface of the metal, permitting it to remain for a sufficient time to act on the metal and produce the desired cleaning effect, then removing the surplus wash along with the 35 products of its action on the metal, and then causing or permitting the metal to dry, thus producing a surface well suited for the reception of paint or other protective coating.

40 Although any metal etching acid may be used with more or less success in making my acid colloidal admixture or scrubbing wash, I prefer to use phosphoric acid because it has rust inhibitive qualities which 45 are very desirable, therefore I will describe my admixture or colloidal scrubbing wash in connection with phosphoric acid although it must be understood that other metal etching acids and acid salts, which produce free 50 hydrogen ions in solution, may be substituted for phosphoric acid without departing from the spirit of the invention.

I have observed that an acid solution, for example, made by mixing 220 gallons of 55 85% phosphoric acid and 641 gallons of

water has a certain speed of cleaning action when metal is dipped into it, but the speed of the cleaning action is greatly reduced when the acid solution is applied as a wash to upright or vertical metallic surfaces. 60 This may be explained by saying that in the case of the immersion of the article to be cleaned in a bath there are a great number of free hydrogen ions in close proximity with the metal surface of the article but in the case of the application of the said solution in the form of a wash to an upright metallic surface the film of the wash adhering to the upright surface is very thin so that there are comparatively few free 65 hydrogen ions in close proximity with the metal. I have further observed that the addition of 82 pounds of gelatine dissolved in 82 gallons of water to the above mentioned acid solution is productive of peculiar results. In the case of a bath the solution acts slower but in the case of a wash the solution acts quicker because in the first case the gelatine interferes with the free movement of the hydrogen ions and in 70 the second case the gelatine causes a material increase in the thickness of the film adhering to the upright metallic surface thus increasing the number of free hydrogen ions in close proximity with the metal and this increase in the number of hydrogen ions more than offsets the restriction of the free movement of the hydrogen ions with the result that the use of gelatine augments 75 the cleaning activity of the wash on upright surfaces. The gelatine may be regarded as a controlling or retarding agent in acid baths since it serves to diminish the cleaning activity but in acid washes it is an accelerating agent and augments the cleaning 80 activity. The following is an example of a cleaning material which produces improved results when applied as a wash:

## Part 1.

|          |            |     |
|----------|------------|-----|
| Gelatine | 82 pounds  | 100 |
| Water    | 82 gallons |     |

## Part 2.

|                     |             |     |
|---------------------|-------------|-----|
| 85% phosphoric acid | 220 gallons | 105 |
| Water               | 641 gallons |     |

Part 1 is made by soaking the gelatine in the water until it softens. The mixture is then heated to 130° F. until the gelatine is 110

thoroughly melted when the mixture is added to Part 2 and the admixture thoroughly stirred.

This forms an excellent cleaner when used according to the process which I have described, but it does not adhere rapidly to an oily surface. To give the cleaner the property of quickly adhering to an oily surface, I add an oil solvent such as wood alcohol, denatured alcohol (ethyl alcohol), fusel oil, butyl alcohol or the like, as shown in the following formula:

*Part 1.*

|    |               |            |
|----|---------------|------------|
| 15 | Gelatine----- | 82 pounds  |
|    | Water-----    | 82 gallons |

*Part 2.*

|    |                          |             |
|----|--------------------------|-------------|
| 20 | 85% phosphoric acid----- | 220 gallons |
|    | Water-----               | 641 gallons |
|    | Butyl alcohol-----       | 50 gallons  |

It will be observed from the above formulas that the gelatine which is a hydrophile (water loving) colloid is converted into a "soluble" colloid (which does not settle out of the admixture, as distinguished from a "solid" colloid such as clay which does settle out) and remains as such in the admixture.

The process of the invention may be commercially carried out by applying the described admixture to the metal, as for instance with a brush; allowing it sufficient time to produce the desired cleaning result, assisting its action with an abrasive during this time if desired; removing what remains of the admixture together with the products of its reaction in any way desired as for example by wiping, blowing off, burning off or washing; and then permitting or causing the metal to thoroughly dry. The metal is then ready to receive the paint or other protective coating.

45 The invention being of a chemical nature I reserve the benefit of the doctrine of equivalents as applied to the construction of patents for such inventions so that it will be evident to those skilled in the art that

modifications and changes may be made in 50 matters of mere form without departing from the spirit of the invention.

I claim:

1. A cleaning wash for use in the preparation of metal for painting which comprises 55 a metal etching acid, a colloid, and a solvent of oil.

2. A cleaning agent for use in the preparation of metal for painting which comprises phosphoric acid, and colloidal gelatine. 60

3. A cleaning wash for use in the preparation of metal for painting which comprises phosphoric acid, colloidal gelatine, and alcohol. 65

4. A cleaning agent for use in the preparation of metal for painting which comprises phosphoric acid, colloidal gelatine, and butyl alcohol.

5. The method of preparing upright metal 70 surfaces for painting which consists in washing it with a metal etching acid in the presence of colloidal gelatine and an oil solvent.

6. The method of preparing an upright metal surface for painting which consists in 75 washing it with phosphoric acid in the presence of colloidal gelatine.

7. The method of preparing upright metal surfaces for painting which consists in washing it with phosphoric acid in the presence 80 of colloidal gelatine and butyl alcohol.

8. The method of preparing an upright metal surface for painting which consists in washing it with a wash comprising phosphoric acid and colloidal gelatine and butyl 85 alcohol, allowing time for the wash to act on the metal, and removing the remainder of the wash together with the products of its action on the metal.

9. The method of preparing an upright 90 metal surface for painting which consists in treating it with an admixture of phosphoric acid, colloidal gelatine and butyl alcohol, assisting the action of the admixture by scrubbing with an abrasive, and removing 95 the remainder of the admixture together with the products of its action.

JAMES H. GRAVELL.